

Dec. 8, 1959

J. CARDELL ET AL

2,916,652

CONTROL OF ELECTRON EMISSION IN CATHODE ASSEMBLIES

Filed Feb. 4, 1955

FIG. 1



EQUATION 2:



EQUATION 3:



FIG. 3

INVENTORS  
JAMES CARDELL  
FREDERICK T. HILL  
BY *Elmer J. Gorn*  
ATTORNEY

## 1

2,916,652

CONTROL OF ELECTRON EMISSION IN  
CATHODE ASSEMBLIES

James Cardell, Auburndale, and Frederick T. Hill, Bedford, Mass., assignors to Raytheon Company, a corporation of Delaware

Application February 4, 1955, Serial No. 486,258

4 Claims. (Cl. 313—346)

This invention relates to electron emission assemblies and, particularly, to the establishment of an efficient relationship between the physical and chemical composition of an electron emitting material, on the one hand, and the physical and chemical composition of the current conducting core, or body, upon which said material is superimposed, on the other.

The invention utilizes the discovery that the emissivity characteristics of a cathode coating, or other electron emitting material, are radically altered by each of two conditions, one physical, the other chemical, to which such emitting material may be subjected. The physical factor is the type of electronic circuit into which the electron emitting element is incorporated, and the chemical factor is the degree of contamination of the core or body material.

Variations in these two factors, it has been discovered, are of such effect upon emissivity as to require, for example, the substitution of a seventy-five percent barium carbonate content in lieu of a twenty percent barium carbonate content for the emission material when the above-described physical and chemical factors are relatively severe. Thus, while a twenty percent barium carbonate content results in most efficient emissivity when the emission element is the coating on a silicon-free cathode of an amplifier tube having a relatively low-temperature cut-off point, with a plate potential of, say, four volts and a heater voltage on the order of 1.7 volts, and with low-field emission, such a relatively low barium carbonate-strontium carbonate ratio does not give comparably good results when the emission element is a coating on an impure (silicon-bearing) nickel cathode incorporated in a tube having a high temperature cut-off level, such as is characteristic of tubes employed in electronic computers, where the cut-off temperature is of such a high value as to establish a high resistance effect at the cathode interface between the core and coating. For such severe duty it has been discovered that raising the barium carbonate-strontium carbonate ratio to 75/25 will provide a beneficial preponderance of barium compound to serve as a buffer agent to check the tendency of the silicon impurities of the cathode core to migrate toward the cathode interface. It is believed that this migration-checking is accomplished by the chemical union of barium-oxide with the migrating silicon molecules, which chemical process can proceed with maximum thoroughness only if the percentage of barium compound in the coating material is high enough to supply the chemical basis for the reaction. It has been found that a barium carbonate percentage well above 50% (as compared with the strontium carbonate percentage), and preferably approaching 75%, is desirable to assure an effective degree of opposition to the silicon migration tendency above described. The result is a maintenance of the interface area in a relatively silicon-free condition, hence in a condition of maximum

## 2

conductivity, with the resistance measurable at the interface dropping to a zero, or near-zero, value.

Other characteristics and advantages flowing from practice of the invention will be apparent upon reference to the following additional explanation, and to the accompanying drawing wherein:

Fig. 1 indicates pertinent chemical reactions, including those occurring when a high-barium coating is applied to a silicon-bearing cathode core;

10 Fig. 2 shows graphically the effect of increases in barium content upon interface resistance, with and without silicon or other impurities in the cathode core;

15 Fig. 3 shows a tube having a cathode to which additional impurities may migrate as heat is applied to all tube parts; and

Fig. 4 is an enlarged sectional view of the cathode assembly of Fig. 3.

The high-barium coating material of the present invention may be prepared, in a small-batch quantity, by 20 weighing out 1351.5 grams of C.P. barium nitrate and 569.4 grams of C.P. strontium nitrate, and placing both materials in a vessel containing ten liters of distilled water for solution therein. After filtering, the clear solution may be placed in a suitable reaction vessel for 25 reaction with the proper quantities of anhydrous sodium carbonate and ammonium carbonate, under heat application, as more fully described in U.S. application Ser. No. 306,879, now Patent No. 2,703,790, filed by M. L. Anderson on August 28, 1952, and assigned to the assignee of the subject application, the reaction products being as indicated in Equation 1 of Fig. 1. The two precipitated carbonates are then washed, filtered, dried, and prepared for use as a cathode coating having a barium-strontium ratio of 75/25, by molecular weight.

30 35 Due to the large preponderance of barium carbonate in the coating material, there will be a correspondingly large preponderance of barium-oxide remaining after the evolution of the  $\text{CO}_2$  gas, in accordance with Equation 2 of Fig. 1. Accordingly, there will be sufficient barium-oxide for chemical union with the silicon impurities of the cathode, to form barium ortho-silicate, as indicated in Equation 3 of Fig. 1. Apparently this chemical union tends to occur in the cathode core before the silicon molecules have had sufficient opportunity to migrate into the interface area and create a dielectric effect at that area. In any event, the effect of the added proportion 40 of barium compound is to change the electrical resistance characteristics of the interface so that the cathode current is transferred across the interface and to the coating emission surface with no resistance being encountered at the interface. This is in sharp contrast to the high interface resistance characterizing other cathode assemblies of the kind described, differing from

50 55 the low resistance assembly only in the percentage of barium carbonate entering into the barium-strontium ratio. The contrast in resistance effects appears to warrant the conclusion that the additional barium content creates the silicon migration-buffering effect above described, by which effect the interface area is freed of the silicon and other impurities, at least to a sufficient degree to reduce the interface resistance to zero, or approximately zero, even with operation of the cathode circuit at a high temperature plateau, such as characterizes tubes used in high-speed pulsing systems.

60 65 70 It has been found that to insure checking of this silicon migration to the degree necessary to reduce the interface resistance to zero, or approximately zero, and to maintain the zero resistance value at the interface even when the tube is subjected to constant operation at the high temperature plateaus characteristic of high-speed pulsing circuits, a barium-strontium molar ratio of at least 75/25

is required. The solid line curve of Fig. 2 (signifying use of a cathode containing silicon impurities in a high temperature cut-off tube, or equivalent severe-duty application) shows that the interface resistance dropped to zero only when the 75/25 ratio of barium carbonate to strontium carbonate was employed, in the particular tube tested. The broken line curve of Fig. 2 (signifying use of a silicon-free cathode in a conventional tube operation with a relatively low cut-off temperature) shows that the interface resistance dropped to zero at a 10 50/50 ratio value, in this particular test.

Fig. 3 shows a type of electron discharge tube in which silicon migration in the indirectly-heated cathode core 11 may be supplemented by additional silicon migration into the core by way of lead-in tab 13, if the latter also contains silicon impurities, as it frequently does. If such a tube is applied to the severe duty represented by the use of high temperature cut-off tubes in computer circuitry, or the like, the effect of such high temperature will be to cause the electrical resistance at the cathode interface 14 (Fig. 4) to have a tendency to be objectionably high, and this in turn will produce a corresponding reduction in emissivity at the surface 15 of the cathode coating, unless the coating contains a barium carbonate preponderance over the strontium carbonate content in a ratio approaching 75/25, as recommended herein. With such a barium preponderance there will be an assurance of an adequate supply of barium oxide for chemical union with all of the migrating silicon, in accordance with Equation 3 of Fig. 1. Such complete chemical absorption of all the migrating silicon will clear the cathode interface of all silicon and related impurities, at least to the degree necessary to drop the interface resistance to a zero, or near-zero, value.

It will be understood, of course, that the triode tube illustrated in Fig. 3 (in which the coiled grid 16, anode 17, and shield 18 are held concentrically spaced by mica disc 12) represents merely one type of tube whose performance can be improved by embodiment of the herein-disclosed invention therein. The invention can be applied with comparable efficiency to electron-emitting diodes, tetrodes, or any other known kind of electron discharge device having a cathode interface resistance problem and a cathode impurity problem such as are inherent in any tube comparable to the tube illustrated in Fig. 3. Likewise, the invention is not limited to the precise proportions, relationships, combinations, and procedures described, as many equivalents will suggest themselves to those skilled in the art. It is accordingly desired that the appended claims be given a broad interpretation commensurate with the scope of the invention within the art.

What is claimed is:

1. In an electron discharge device adapted for high temperature level operation, a cathode comprising a core 55 of conducting material having silicon impurities therein,

and a coating on said core comprising a mixture of oxygen-bearing barium and strontium compounds, in which the ratio of barium to strontium is substantially seventy-five to twenty-five percent by molecular weight, whereby a low-resistance interface intermediate said core and said coating including the complex silicates of barium and strontium is formed, thereby enabling the free flow of electrons from said cathode.

2. In an electron discharge device adapted for high temperature level operation, a cathode comprising a core of conducting material having silicon impurities therein, and a coating on said core comprising alkaline rare earth metal oxides including barium and strontium, in which the ratio of barium to strontium by molecular weight is in a range effective to reduce the interface resistance between said core and said coating to a value of substantially zero, thereby enabling the free flow of electrons from said cathode, said interface intermediate said core and said coating including the complex silicates of said rare earth metals.

3. In combination, an electron discharge device adapted for high temperature level operation, said device having a cathode comprising a core of conducting material having silicon impurities therein, a layer of electron emissive material on said core, said layer comprising a mixture of a barium compound and a strontium compound wherein the barium compound is present in a proportion substantially seventy-five percent by molecular weight, and means operative to subject said electron discharge device to high temperature level operation.

4. In an electron discharge device adapted for high temperature level operation, a cathode comprising a core of conducting material having silicon impurities therein, and a layer of electron emissive material on said core, said layer comprising a mixture of a barium compound and a strontium compound wherein the ratio of barium to strontium is substantially seventy-five percent to twenty-five percent by molecular weight.

#### References Cited in the file of this patent

##### UNITED STATES PATENTS

|           |                 |               |
|-----------|-----------------|---------------|
| 1,542,385 | Harris          | June 16, 1925 |
| 1,813,320 | Schaefer et al. | July 7, 1931  |
| 1,870,951 | Fredenburgh     | Aug. 9, 1932  |
| 1,961,122 | Lowry           | May 29, 1934  |
| 1,981,245 | Pearcy          | Nov. 20, 1934 |
| 2,246,162 | Benjamin        | June 17, 1941 |
| 2,306,290 | Widell          | Dec. 22, 1942 |
| 2,535,999 | Bouchard        | Dec. 26, 1950 |
| 2,566,115 | Bounds          | Aug. 28, 1951 |
| 2,703,790 | Anderson        | Mar. 8, 1955  |

##### FOREIGN PATENTS

|         |               |               |
|---------|---------------|---------------|
| 535,659 | Canada        | Jan. 8, 1957  |
| 710,648 | Great Britain | June 16, 1954 |